

# UNITED STATES PATENT OFFICE.

HUGH S. COOPER, OF CLEVELAND, OHIO, ASSIGNOR TO THE ELECTRO METALS PRODUCTS COMPANY, OF CLEVELAND, OHIO.

## METAL ALLOY.

1,229,037.

Specification of Letters Patent.

Patented June 5, 1917.

No Drawing.

Application filed August 14, 1915. Serial No. 45,526.

*To all whom it may concern:*

Be it known that I, HUGH S. COOPER, a citizen of the United States, residing at Cleveland, in the county of Cuyahoga and State of Ohio, have invented certain new and useful Improvements in Metal Alloys, of which the following is a specification.

My invention appertains to a metal alloy adapted to be used as a substitute for platinum in the electrical art, as in coils, magnetos and all vibrating instruments, and the invention consists of a composition of silver and other metals which is ductile, and malleable, and of comparatively high melting point, good electrical conductivity, great hardness, non-oxidizing, and producible at a low cost.

In all compositions of alloys known to me in which silver enters, copper is also used but I find that this composition oxidizes very readily making it useless for electrical contact purposes, especially where the contact is exposed to high temperatures and severe usage. I also find that it is not practicable to use silver alone as it is too soft and the melting point is not high enough. However, silver is a good electrical conductor and relatively cheap as compared with platinum and when alloyed in proper proportions with other metals as hereinafter described serves as an excellent substitute for platinum. One such composition comprises silver, palladium and cobalt, in substantially the following proportions: seventy per cent. of silver, twenty-five per cent. of palladium, and five per cent. of cobalt. Platinum may be substituted for the palladium with equally good

results, and nickel for the cobalt, but I prefer palladium as it may be obtained at a lower cost than platinum. I also prefer 40 cobalt as I find it resists oxidization at a higher temperature than nickel, and it also makes a harder alloy. In this alloy I use as little of platinum or palladium as possible consistent with the durability and lasting qualities of the product, and I also find that three to five per cent. of cobalt or nickel is sufficient to furnish the hardness necessary.

What I claim is:

1. An alloy for electrical uses, comprising silver and one or more of the metals of the platinum group and a metal of the cobalt-nickel group in substantially the proportions stated.

2. An alloy for electrical uses containing silver, palladium, and a metal of the cobalt-nickel group in the proportions substantially set forth.

3. An alloy for electrical contact purposes 60 composed of silver, palladium, and cobalt in approximately the proportions stated as to make the alloy hard, heat resisting, non-oxidizing and a good electrical conductor.

4. A metal alloy composed of seventy per 65 cent. of silver, twenty-five per cent. of palladium, and five per cent. cobalt.

In testimony whereof I affix my signature in presence of two witnesses.

HUGH S. COOPER.

Witnesses:

J. W. FRASER,  
R. B. MOSER.